

## UNITED STATES PATENT OFFICE

2,116,432

## GETTER FOR VACUUM DEVICES

Daniel S. Gustin, Bloomfield, N. J., assignor, by  
mesne assignments, to Westinghouse Electric  
and Manufacturing Company, East Pittsburgh,  
Pa., a corporation of Pennsylvania

No Drawing. Original application October 21,  
1932, Serial No. 638,995. Divided and this ap-  
plication May 6, 1936, Serial No. 78,169

14 Claims.

(Cl. 176—2)

This invention relates to the manufacture of  
vacuum devices and, more particularly, to the  
evacuation of incandescent electric lamps, and  
is a division of my application Serial No. 638,995  
5 filed October 21, 1932, now Patent 2,042,935 dated  
June 2, 1936 and owned by the assignee of the  
present application.

The practice of making incandescent electric  
lamps includes the operation of removing the gas  
10 from the bulb which is accomplished by the use  
of mechanical means, such as vacuum pumps,  
and in subsequently removing any residual gas  
by means of suitable substances termed "getters".  
The present invention is directed to an improved  
15 form of getter or clean-up agent to bring about  
a more complete clean-up or removal of residual  
gas in vacuum devices such as incandescent elec-  
tric lamps, radio tubes, and the like. When the  
term getter is used in the following specification  
20 and claims, it is to be construed as a substance  
capable of removing the greater portion or, as  
near as possible, all of the residual gas.

Many substances and combinations of sub-  
stances have been employed as clean-up agents  
25 and one form of getter which has been success-  
fully used contains 100 parts by weight of cryolite  
and 13 parts by weight of phosphorus.

When using such a getter, it is applied in the  
30 form of a paste or liquid to the filament. When  
the filament is heated the getter is driven off.  
According to the accepted theory, the cryolite is  
precipitated to the surface of the bulb and re-  
35 mains there to receive particles resulting from  
the vaporization of the filament. The cryolite  
presents an irregular serrated surface so that the  
solid or opaque particles are widely distributed  
and become ineffective in obscuring the light or,  
40 in other words, the cryolite prevents blackening  
of the bulb.

The phosphorus is in the form of red phos-  
phorus which, when heated, is converted to yellow  
45 phosphorus in the form of a vapor. This vapor is ionized by the electric discharge between  
the lead wires of the lamp or between the coils  
of the filament when such type of filament is  
employed. The ionization converts the yellow  
50 phosphorus vapor to red phosphorus which, dur-  
ing conversion, causes a physical chemical re-  
action with the residual gas and removes the  
same in the sense that such gas is taken up by  
the red phosphorus particles which are widely  
55 distributed on the wall of the bulb and rendered  
invisible by reason of the cryolite which receives  
them.

I have found that the residual gas may be

completely removed or rendered ineffective if the  
ionization of the phosphorus or other vapor is  
increased by a more copious supply of electrons.

It is an object of the present invention, there-  
fore, to provide a getter capable of promoting  
5 ionization.

Another object of the invention is to provide a  
getter containing a thermionically active mate-  
rial to promote the clean-up action of the getter.

A further object of the invention is to improve  
the vacuum in a sealed envelope by providing a  
10 substance for increasing the ionization of a va-  
porized constituent of a getter.

Other objects and advantages of the invention  
will be apparent from the following description. 15

When practicing the present invention I have  
found that good results are obtained by using  
getter composed of 100 parts by weight of cryolite  
and 13 parts by weight of phosphorus to which  
may be added 1.3% or less of a thermionically  
20 active substance such as barium carbonate.  
These substances may be thoroughly mixed with  
a binder of nitrocellulose to provide a paste or  
it may be in liquid form so that the getter may be  
sprayed onto a filament. I have found that the  
25 barium oxide resulting from the heating increases  
the electron emissivity and the carbon dioxide  
increases the amount of gas to be ionized.

It is to be understood that the present inven-  
tion in its broadest aspects contemplates the use  
30 of a material to increase the electron flow in the  
presence of a clean-up agent. Barium or other  
alkaline earth metals may be used such, for ex-  
ample, as strontium, or the oxides or compounds  
35 of these substances may be used. Furthermore,  
the material for increasing or promoting ioniza-  
tion may be used with other getter materials in  
which ionization is effective to clean up residual  
gases. As an alternative of the above getter  
40 composition, I may use inorganic halogen com-  
pounds such as fluorides or double fluorides or  
sodium chloride and similar halogen compounds.  
By adding to such getters a substance such as  
45 barium or other substances to promote electron  
emission, the resultant ionization improves the  
vacuum by the removal of the residual gas.

By reason of the present invention a clean-up  
agent or getter is provided wherein the thermioni-  
cally active material is a part of the mixture used.  
In the case of a cryolite phosphorus getter, for  
50 example, the cryolite performs its function as does  
the phosphorus while the added substance, by  
reason of the more copious supply of electrons  
furnished, promotes ionization thus making the  
clean-up action more complete, resulting in a 55

higher degree of vacuum than had heretofore been possible.

Although a preferred embodiment of the invention is shown and described herein, it is to be understood that modifications may be made without departing from the spirit and scope of the invention as set forth in the appended claims.

I claim:

1. A getter for a vacuum device comprising phosphorus and barium oxide.
2. A getter for a vacuum device comprising cryolite, phosphorus and barium oxide.
3. A substance for removing residual gases from a sealed container, said substance comprising phosphorus, cryolite and an alkaline earth metal compound.
4. A substance for removing residual gases from a sealed container, said substance comprising phosphorus, cryolite and a barium compound.
5. A getter for a vacuum device comprising phosphorus and a barium compound.
6. A getter for a vacuum device comprising cryolite, a barium compound, and a clean up agent.
7. A getter for a vacuum device comprising cryolite, barium oxide, and a clean up agent.
8. A getter for a vacuum device comprising phosphorus and an alkaline earth metal compound.
9. A getter for a vacuum device comprising cryolite, an alkaline earth metal compound, and a clean up agent.

10. A clean-up agent for the residual gas in a sealed container, said agent comprising a substance vaporizable when heated to combine with said gas and an alkaline earth metal compound for supplying a copious amount of electrons to promote ionization of said vapor to improve its clean-up action.

11. A clean-up agent for the residual gas in a sealed container, said agent comprising a substance vaporizable when heated to combine with said gas and a barium oxide for supplying a copious amount of electrons to promote ionization of said vapor to improve its clean-up action.

12. A clean-up agent for the residual gas in a sealed container, said agent comprising a substance vaporizable when heated to combine with said gas and a barium compound for supplying a copious amount of electrons to promote ionization of said vapor to improve its clean-up action.

13. A clean-up agent for the residual gas in a sealed container, said agent comprising phosphorus to combine with said gas and an alkaline earth metal compound for supplying a copious amount of electrons to promote ionization of said phosphorus to improve its clean-up action.

14. A getter for an incandescent electric lamp comprising an alkaline earth metal compound and a clean-up agent applied to the filament of said lamp for temporarily promoting ionization of said clean-up agent when said filament is flashed.

DANIEL S. GUSTIN.